

## UNITED STATES PATENT OFFICE

2,185,262

COMPOUND FOR AND PROCESS OF SURFACE  
FINISHING METALLIC ARTICLES

Joseph Lupo, Jr., Bronx, N. Y.

No Drawing. Application April 9, 1938,  
Serial No. 201,107

9 Claims. (Cl. 51—278)

This invention is for an improved process of finishing the surfaces of metallic parts or articles, such as zinc die castings, brass castings, steel, nickel, gold, stainless steel, platinum and silver stampings or castings by a mass tumbling method.

The invention broadly comprehends a dry process for cutting down and smoothening the surfaces of metal articles by tumbling the same with hard, bony pellets and an abrasive compound composed of an abrasive material and lubricating and adhesive vehicles.

The invention further resides in a process of the character indicated in which the metal articles are tumbled in a dry mixture of hard, bony pellets, absorptive, fibrous fragments and an abrasive compound composed of an abrasive material and lubricating and adhesive vehicles.

The invention also comprehends an improved tumbling process for cutting down and smoothening the surfaces of the articles so as to remove tool, grinding and sand marks or other defects; for producing a mat or frosted finish where the articles are to be immediately plated; for obtaining a temporarily burnishing or high luster finish, while coating or protecting the surfaces against tarnishing, rusting, corrosion or other discolorations if the articles are to be subsequently but not immediately plated and for producing a permanent high luster finish if the articles are not to be plated.

The invention provides a process and compounds for the finishing of the surfaces of metallic articles or parts whereby the finishing may be more economically accomplished than with the hand process heretofore employed by virtue of which process a superior and more uniform surface finish is obtained, while eliminating detrimental overheating of the metal resulting in burns and spots which frequently are not closed until the surface is plated.

As a further advantage the articles processed by the compounds and method of this invention are positively devoid of dangerous sharp edges

and acids and require no subsequent washing or cleansing with expensive metal cleaners.

In carrying out the invention the metal articles are preferably tumbled in a tumbling machine with hard bony pellets together with a compound including a hard coarse abrasive to effect a cutting down of the surfaces thereof so as to remove tool, grinding or sand marks or other defects. After the cutting down of the metal articles, if the same are to be polished or burnished, they are tumbled with hard bony pellets and a compound including a hard fine abrasive and thereafter if it is desired to impart a high luster to the metal articles, the same are tumbled with absorptive fibrous fragments coated with a compound including a flour abrasive.

The hard bony pellets employed in the cutting down and polishing operations preferably consist of vegetable ivory chips, bone chips, synthetic resin chips or hard tree root chips, while the compound includes an abrasive, a lubricating vehicle and an adhesive vehicle.

For metal parts which are devoid of fine holes or threads, the abrasive compound is preferably applied to the surface of the absorptive fibrous fragments, such as a sawdust, wood chips or leather particles by coating the same with the lubricating vehicle which may be kerosene or any other equivalent light thin mineral oil, and then applying thereto the abrasive or cutting material such as ground pumice, emery, carborundum, precipitated chalk, infusorial earth, finely ground tripoli or other flour abrasive which is bonded to the fibrous fragments by the adhesive vehicle which may consist of tallow, petrodatum or other fatty substances.

The tumbling barrel is approximately half filled with the metal articles, pellets or pellets and fibrous fragments in the proportion of approximately one part of metal articles to two parts of the pellets and fragments or two and one-half parts thereof by volume so as to provide a body in which the metal articles are embedded and individually surrounded to avoid sharp impact and rough tumbling of the metal articles.

against each other, thus preventing marring or scratching of the same, while the pellets and fibrous fragments effect a uniform abrading action of the abrasive material against the entire surface of each of the articles.

In the cutting down operation for removing tool, grinding or sand marks or other defects in metal articles, which are devoid of fine holes or threads, it has been found that practical and

10 satisfactory results are expeditiously obtained by charging the tumbling barrel in the following proportions by volume:

|                                                                                                               | Per cent |
|---------------------------------------------------------------------------------------------------------------|----------|
| 15 Hard bony pellets such as vegetable ivory chips, bone chips, synthetic resin chips or hard tree root chips | 65       |
| Abrasive compound                                                                                             | 10       |
| Metal articles                                                                                                | 25       |

20 The abrasive compound in this operation preferably consists of the following ingredients by volume:

|                                                                                                        | Per cent |
|--------------------------------------------------------------------------------------------------------|----------|
| 25 Absorptive fibrous fragments, such as hard wood granulated sawdust, wood chips or leather fragments | 60       |
| Kerosene or other equivalent light thin mineral oil                                                    | 10       |
| Abrasive material and lubricating and adhesive vehicles                                                | 30       |

The abrasive material and vehicles preferably include the following ingredients by volume:

|                                                                                                              | Per cent |
|--------------------------------------------------------------------------------------------------------------|----------|
| 35 Hard coarse abrasive, such as ground pumice, emery or carborundum of 180 to 200 mesh                      | 24       |
| Lubricating vehicle, such as kerosene or other equivalent light thin mineral oil                             | 45       |
| 40 Adhesive vehicle, such as tallow, degras, mineral grease, chicken or animal fat or other fatty substances | 18       |
| Adhesive vehicle, such as petrolatum or heavy mineral oil having a high viscosity                            | 30       |

45 When the metal articles have fine holes or threads in which the fibrous fragments may become caked therein, the tumbling barrel is charged in the following proportions by volume:

|                                                                                                                | Per cent |
|----------------------------------------------------------------------------------------------------------------|----------|
| 50 Hard bony pellets, such as vegetable ivory chips, bone chips, synthetic resin chips or hard tree root chips | 75       |
| Abrasive material and vehicles                                                                                 | 1        |
| Metal articles                                                                                                 | 24       |

55 It will be observed that in this charging the absorptive fibrous fragments, such as the sawdust, wood chips or leather particles are eliminated in order to prevent clogging or caking of the fine holes or threads.

60 When the absorptive fibrous fragments are employed in the operation, the same are coated with the kerosene or other equivalent light thin mineral oil, after which the abrasive material is applied thereto and then the adhesive vehicle, such as tallow and petrolatum or their equivalents applied over the surface of the abrasive to bond the same to the fibrous fragments.

65 When the absorptive fibrous fragments are not employed in the operation, the abrasive material is obtained by mixing together the aforesaid quantities of kerosene, tallow and petrolatum or their equivalents and then adding the proportion of abrasive specified and the entire mass mixed into a homogeneous mash.

75 In the operation of polishing or burnishing

metal articles which do not have fine holes or threads, after the same have been cut down by the operation described, the tumbling barrel is preferably charged in the following proportions by volume:

|                                                                                                             | Per cent |
|-------------------------------------------------------------------------------------------------------------|----------|
| Hard bony pellets, such as vegetable ivory chips, bone chips, synthetic resin chips or hard tree root chips | 65       |
| Abrasive compound                                                                                           | 10       |
| Metal articles                                                                                              | 25       |

The abrasive compound in this operation preferably consists of the following ingredients by volume:

|                                                                                                     | Per cent |
|-----------------------------------------------------------------------------------------------------|----------|
| Absorptive fibrous fragments, such as hard wood granulated sawdust, wood chips or leather fragments | 42       |
| Kerosene or other equivalent light thin mineral oil                                                 | 10       |
| Abrasive such as 320 to 400 mesh pumice, emery or carborundum                                       | 20       |
| Abrasive material and lubricating and adhesive vehicles                                             | 28       |
|                                                                                                     | 25       |

The abrasive material and lubricating and adhesive vehicles in this operation preferably include the following ingredients by volume:

|                                                                                                           | Per cent |
|-----------------------------------------------------------------------------------------------------------|----------|
| Hard fine abrasive, such as pumice, emery or carborundum                                                  | 30       |
| Kerosene or other equivalent light mineral oil                                                            | 19       |
| Adhesive vehicle such as tallow, degras, red oil, steric acid or other fatty mineral or animal substances | 47       |
| Adhesive vehicle, such as petrolatum or other heavy mineral oil                                           | 35       |
|                                                                                                           | 23       |
|                                                                                                           | 11       |
|                                                                                                           | 40       |

In the polishing and burnishing operation, the absorptive fibrous fragments having an outside coating of the adhesive material, such as the tallow and petrolatum or other equivalents, come into contact with the hard bony pellets and the metal articles when tumbled together therewith in a tumbling barrel so as to intimately coat the surfaces thereof with the said vehicle and the abrasive material thereby exposing the lubricating vehicle constituting the inner layer on the fibrous fragments so that by the rolling contact of the metal articles with the hard bony pellets and the relatively softer fibrous fragments, the abrasive material effects a polishing of the metal articles while the lubricating and adhesive vehicles prevent overheating thereof during the tumbling operation.

For metal parts having fine holes or threads in which the absorptive fibrous fragments, such as the sawdust, wood chips or leather parts may become caked therein, the tumbling barrel is preferably charged in the following proportions by volume:

|                                                                                                             | Per cent |
|-------------------------------------------------------------------------------------------------------------|----------|
| Hard bony pellets, such as vegetable ivory chips, bone chips, synthetic resin chips or hard tree root chips | 75       |
| Abrasive material and vehicles                                                                              | 1        |
| Metal articles                                                                                              | 24       |
|                                                                                                             | 70       |

For imparting a high luster to metal articles which do not have fine holes or threads, after the same have been subjected to the cutting down, polishing or burnishing operations, the

tumbling barrel is preferably charged in the following proportions by volume:

|                                            | Per cent |
|--------------------------------------------|----------|
| Absorptive fibrous fragments, such as wood | 75       |
| 5 pegs                                     | 1        |
| Abrasive compound                          | 24       |

The abrasive compound in this operation preferably consists of the following ingredients by volume:

|                                                                                | Per cent |
|--------------------------------------------------------------------------------|----------|
| Absorptive fibrous fragments, such as sawdust, wood chips or leather fragments | 72       |
| 15 Lubricating vehicle such as red oil                                         | 1        |
| Abrasive material and lubricating and adhesive vehicles                        | 27       |

The abrasive material and vehicles in this operation preferably consists in the following ingredients by volume:

|                                                                                                           | Per cent |
|-----------------------------------------------------------------------------------------------------------|----------|
| Fine or flour abrasive, such as precipitated chalk, infusorial earth, tripoli of 500 to 800 mesh          | 23       |
| 25 Lubricating vehicle, such as red oil                                                                   | 42       |
| Adhesive vehicle, such as tallow, degras, mineral grease, chicken or animal fat or other fatty substances | 25       |
| Adhesive vehicle, such as heavy thick mineral oil                                                         | 10       |

For metal parts having fine holes or threads in which the sawdust may become caked therein, the tumbling barrel is preferably charged in the following proportions:

|                                | Per cent |
|--------------------------------|----------|
| Wood pegs                      | 75       |
| Abrasive material and vehicles | 1        |
| Metal articles                 | 24       |

40 As a substitute for the kerosene or light thin mineral oil in the abrasive compound for the cutting down and smoothening operations, the following may be employed:

|                        | Per cent |
|------------------------|----------|
| 45 Trisodium phosphate | 7        |
| Low grade soap         | 15       |
| Tallow                 | 21       |
| Water                  | 57       |

50 In place of the kerosene and tallow ingredients in the abrasive material and vehicles in the cutting down and smoothening operations, the following may be employed:

|                      | Per cent |
|----------------------|----------|
| Trisodium phosphate  | 23       |
| 55 Low grade soap    | 10       |
| Water                | 52       |
| Tallow or animal fat | 15       |

What is claimed is:

- 60 1. The process for finishing the surfaces of metal articles which consists in tumbling the same in a dry mass composed of vegetable ivory chips and an abrasive compound including an abrasive material and lubricating and adhesive vehicles.
- 65 2. The process for finishing the surfaces of metal articles which consists in tumbling the

same in a dry mass composed of hard bony pellets, absorptive fibrous fragments, and an abrasive compound consisting of abrasive material and lubricating and adhesive vehicles.

3. The process for finishing the surfaces of metal articles which consists in tumbling the same in a dry mass composed of hard bony pellets, absorptive fibrous fragments, and an abrasive compound consisting of abrasive material and lubricating and adhesive vehicles coated upon the fibrous fragments with the abrasive material disposed between the lubricating and adhesive vehicles.

4. The process for finishing metal articles which consists in first tumbling the same in a dry mass composed of vegetable ivory chips and an abrasive compound including a hard coarse abrasive and lubricating and adhesive vehicles to effect a substantial cutting down and smoothening of the surfaces of the metal articles and then tumbling the same in a dry mass composed of vegetable ivory chips and an abrasive compound including a hard fine abrasive and lubricating and adhesive vehicles to effect a polishing and burnishing of the surfaces thereof.

5. The process for finishing metal articles which consists in first tumbling the same in a dry mass composed of vegetable ivory chips and an abrasive compound including a hard coarse abrasive and lubricating and adhesive vehicles to effect a substantial cutting down and smoothening of the surfaces of the metal articles and then tumbling the same in a dry mass composed of vegetable ivory chips and an abrasive compound including a hard fine abrasive and lubricating and adhesive vehicles to effect a polishing and burnishing of the surfaces thereof, and thereafter tumbling the same in a dry mass composed of absorptive fibrous fragments and an abrasive compound including a flour abrasive and lubricating and adhesive vehicles to impart a high luster to the surfaces thereof.

6. The process for finishing the surfaces of metal articles which consists in tumbling the same in the approximate proportion by volume of 25% of metal articles with 75% of a dry mass composed of vegetable ivory chips and an abrasive compound including an abrasive material and lubricating and adhesive vehicles.

7. A tumbling material for finishing metal articles comprising a dry mass composed of hard bony pellets, absorptive fibrous fragments, and an abrasive compound including abrasive material and lubricating and adhesive vehicles.

8. A tumbling material for finishing metal articles comprising a dry mass composed of hard bony pellets, absorptive fibrous fragments, and an abrasive compound including abrasive material and lubricating and adhesive vehicles carried by the fibrous fragments.

9. A tumbling material for finishing metal articles comprising a dry mass composed of vegetable ivory chips, and an abrasive compound including abrasive material and lubricating and adhesive vehicles.

JOSEPH LUPO, JR.